

## [54] PROCESS FOR THE DYEING OF TEXTILE MATERIAL AND APPARATUS FOR CARRYING OUT THE PROCESS

[75] Inventors: Hans Scheidegger, Binningen, Switzerland; Hermann Flensberg, Weil am Rhein, Fed. Rep. of Germany; Roland Bauhofer, Böckten, Switzerland

[73] Assignee: Ciba-Geigy Corporation, Ardsley, N.Y.

[21] Appl. No.: 230,150

[22] Filed: Jan. 30, 1981

## Related U.S. Application Data

[63] Continuation of Ser. No. 935,830, Aug. 22, 1978, abandoned, which is a continuation of Ser. No. 755,699, Dec. 30, 1976, abandoned.

## [30] Foreign Application Priority Data

Jan. 6, 1976 [CH] Switzerland 51/76

[51] Int. Cl.<sup>3</sup> D06P 1/39; D06P 3/06

[52] U.S. Cl. 8/636; 8/929; 8/158

[58] Field of Search 8/633, 634, 620, 636, 8/929

## [56] References Cited

## U.S. PATENT DOCUMENTS

|           |         |                |       |
|-----------|---------|----------------|-------|
| 2,900,218 | 8/1959  | Gray           | 8/602 |
| 3,317,271 | 5/1967  | Mecco          | 8/929 |
| 3,352,624 | 11/1967 | Harding et al. | 8/481 |
| 3,627,473 | 12/1971 | Eltonhead      | 8/531 |

3,936,268 2/1976 Papalos 8/589

## FOREIGN PATENT DOCUMENTS

|         |         |                      |
|---------|---------|----------------------|
| 2361491 | 12/1963 | Fed. Rep. of Germany |
| 161381  | 6/1971  | Fed. Rep. of Germany |
| 605258  | 7/1948  | United Kingdom       |
| 1404545 | 9/1975  | United Kingdom       |
| 1450216 | 9/1976  | United Kingdom       |
| 1458632 | 12/1976 | United Kingdom       |

## OTHER PUBLICATIONS

Nitschke, G., VEB Verlag Technik 1954, pp. 63-66.  
Weckler, G., Meilland 11, 1963, pp. 1224-1239.

Primary Examiner—Maria Parrish Tungol  
Attorney, Agent, or Firm—Edward McC. Roberts

## [57]

## ABSTRACT

Described is a process for the dyeing of textile material by the exhaust method, whereby the dyeing is commenced at a pH value of between 6 and 12 and terminated at a pH value of between 3 and 7, which process is characterized in that during dyeing the pH value is lowered, by the addition of an inorganic acid, by at least 1 unit of pH value; and that subsequent to the dyeing the exhausted bath, after the addition of alkali, dye and, if required, further auxiliaries, is optionally used afresh for dyeing.

Furthermore an apparatus for carrying out this process is described which consists of a dyeing aggregate having a liquor-circulating system which contains at least one pH-measuring point as well as at least one dosing device.

10 Claims, 4 Drawing Figures

Fig. 1



Fig. 2





Fig. 3

Fig. 4



PROCESS FOR THE DYEING OF TEXTILE  
MATERIAL AND APPARATUS FOR CARRYING  
OUT THE PROCESS

This is a Continuation of application Ser. No. 935,830 filed on Aug. 22, 1978, now abandoned which in turn is a Continuation of application Ser. No. 755,699 filed Dec. 30, 1976, now abandoned.

The present invention relates to a process for the level, rational, reliable and environmentally favourable dyeing of textile material by the exhaust method, to the application of the process to textile material made principally from fibres that can be dyed with anionic dyes, such as synthetic polyamide or wool, to the textile material dyed by this process, as well as to the apparatus for carrying out the process.

Textile material that can be dyed with anionic dyes, such as synthetic polyamide or wool, is usually dyed from a more or less buffered, slightly alkaline, neutral or weakly acid bath. Towards the end of dyeing, there is sometimes added an organic acid, such as acetic acid; the degree of exhaustion is certainly improved as a result, but problems frequently arise with regard to the levelness of the dyeings.

The use of sulphuric acid is not advised because, although the degree of exhaustion is further improved as a result, the risk of obtaining unlevel dyeings by virtue of blocking effects is particularly great [see H. U. Schmidlin: Vorbehandlung und Färben von synthetischen Faserstoffen (Preliminary treatment and dyeing of synthetic fibre materials), Publishers: Schweizerische Vereinigung von Färbereifachleuten (Swiss Association of Dyeing Specialists), Basle 1968].

The German 'Offenlegungsschrift' No. 2,354,728 discloses a process for dyeing wool and polyamide, wherein dyeing is commenced at a pH value of 7.5 to 11 and completed at a pH value of 4 to 6.5. The change in the pH value is achieved by addition of lactones as acid donators, which during the dyeing process are continuously hydrolysed. In this Offenlegungsschrift the use of free acids instead of the lactones is not advised since the levelness would be impaired, particularly in the case of light dyeings.

These known processes possess however the great disadvantage that after each dyeing there have accumulated large amounts of waste liquor, which have to be freed from dyes and in some cases from textile auxiliaries. A re-utilization of the dyebath is possible only with difficulty because too much of the dyes, auxiliaries and unconsumed acid donators remain in the bath after dyeing. Furthermore, because of the weak organic acid in conjunction with the alkali necessary for obtainment of the initial pH value, there would be formed in the dyebath a buffer system, so that with renewed acidification, the final pH value could be obtained only by the addition of considerably greater amounts of acid donators.

It has now been found that it is possible, without extra dyeing or analytical expenditure, with the attainment of very reproducible dyeings, to repeatedly use the dyebath if measures are taken to ensure that the dyes are absorbed as completely as possible onto the textile material. This is achieved by lowering the pH value of the dyebath by the addition of a strong acid during the course of dyeing. The difficulties with respect to the levelness of the dyeings can be surprisingly avoided by virtue of the addition of acid being made gradually.

The process according to the invention offers a considerable advance in the art. The amount of waste liquor is greatly reduced by the repeated use of the dyebath. Moreover, in consequence of the better degree of exhaustion the waste liquors contain an amount of dye that is appreciably less than that contained by the baths remaining after the customary processes, and there are required no buffer systems containing phosphates or borates, which are ecologically unsafe. As a consequence of the use of inorganic acids instead of organic acids, it is also possible to reduce the oxygen requirement for the biological purification of the waste liquors. The result is therefore a considerable saving of water, of dyes and of other auxiliary chemicals, as well as of energy, since the exhausted dyebaths on repeated use do not have to be reheated each time from room temperature to the dyeing temperature. It is merely necessary to compensate for cooling which, even with the use of a device for hot withdrawal, occurs whilst the material is being changed.

In addition, the process according to the invention has the particular advantage that dyeings are obtained which, even after repeated use of the bath, have very good reproducibility with regard to depth of colour and shade; and, furthermore, the results of small-scale tests (laboratory dyeings) can be excellently related to dyeings on a commercial scale.

Because of the high degree of exhaustion of the dyes, a rinsing process is in many cases unnecessary, which constitutes a further rationalisation.

The present invention hence relates to a process for the level, rational, reliable and environmentally favourable dyeing of textile material by the exhaust method, whereby the dyeing is commenced at a pH value of between 6 and 12 and terminated at a pH value of between 3 and 7, which process is characterised in that at the commencement of dyeing the initial pH value is adjusted if necessary by the addition of strong alkali; that during dyeing the pH value is lowered, by the addition of a strong inorganic acid, by at least 1 unit of pH value; and that subsequent to the dyeing the exhausted bath, after the addition of alkali, dye and, if required, further auxiliaries, is optionally used afresh for dyeing.

A preferred embodiment of the invention comprises commencing the dyeing at a pH value of 7.0 to 10.0 and terminating it at a pH value of 3.5 to 6. The pH value to be applied depends essentially on the type and concentration of the dyes, on the substrate and on the type of dyeing aggregate. These pH values are known or are readily determinable.

To the dyebath are subsequently added alkali, optionally auxiliaries, and dyes and the dyebath is used afresh for dyeing. Suitable alkalies are salts of strong bases with weak acids, e.g. ammonium carbonate, sodium carbonate or potassium carbonate or ammonium hydrogen carbonate, sodium hydrogen carbonate or potassium hydrogen carbonate, as well as preferably strong bases such as NaOH or KOH, which are added optionally all at once, portionwise or preferably in controlled amounts.

The lowering of the pH value during dyeing is effected by the addition of a strong inorganic acid of which the  $pK_a$  value at 20° C. is below 3.8. Suitable inorganic acids are, in particular, nitric acid, hydrochloric acid and especially sulphuric acid.

The acid is added to the dye bath, preferably after attainment of the dyeing temperature, in such a manner that a level dyeing results.

The addition of acid can be made, for example, within 5 to 90 minutes in 5 to 15 equal portions, or continuously, e.g. with a constant rate of feed. It is also possible to feed in the acid in 2 or more phases, the rate of flow for each phase being constant but differing from one phase to another; and also to have pauses in between during which no addition of acid is made. It is advantageous however to perform the addition of acid by means of a suitable regulating and/or control device, e.g. in such a way that there occurs a predetermined pH variation relative to time and /or to temperature. This pH variation can follow one or more linear and/or 15 nonlinear gradients.

Textile materials made up of material dyeable with anionic dyes can be dyed by the process according to the invention. The process can be used, in particular, for dyeing natural polyamides, such as wool or silk, or 20 synthetic polyamides. Such synthetic polyamides are, e.g., polymers of  $\epsilon$ -caprolactam (polyamide 6), condensation products from hexamethylenediamine and adipic acid (polyamide 6.6) or sebacid acid (polyamide 6.10), or mixed condensation products, e.g. from hexamethyl- 25 enediamine, adipic acid and  $\epsilon$ -caprolactam (polyamide 6.6/6), also the polymerisation products from  $\epsilon$ -caprolactam or from  $\omega$ -aminoundecanoic acid (polyamide 11), and modified polyamide types. Also applicable are mixtures of these fibres, and also of wool and synthetic polyamide. The make-up of these fibre materials can be very varied; they can be for example in the form of loose material, yarn in all forms of make-up, fabrics, 30 knitted fabrics, knitwear, fibre fleece materials and, in particular, carpets.

Dyes usable according to the invention are preferably anionic, water-soluble or at least dispersible in water. They can be reactive or preferably nonreactive, i.e. they are able or not able to form with the fibre material a covalent bond, and they can belong to different classes 40 of dyes. They are, for example, salts of metal-free or heavy-metal-containing mono-, dis- or polyazo dyes, including the formazan dyes, as well as anthraquinone, nitro, triphenylmethane and phthalocyanine dyes. Of interest are also the 1:2 metal-complex dyes. The anionic character of these dyes can be caused by metal-complex formation alone and/or by acid salt-forming 45 substituents, such as carboxylic acid groups, sulphuric acid groups and phosphoric acid ester groups, phosphoric acid groups or sulphonate acid groups.

In addition, the dye bath can contain disperse dyes and/or cationic dyes. All these dyes must be essentially stable in the pH range in which dyeing is performed.

For this form of application, namely the dyeing of, e.g., differentially-dyeing polyamide carpet material or possibly of other types of fibres, the process has considerable technical advantages. Since, as is known, the migration of dyes and also the differentiation effect, which are responsible for surface levelness, are very greatly dependent on the pH value, and since for these two phenomena also different pH values are optimum, the selection of the pH value in the process applied hitherto has been very limited by the choice of the buffer systems available. Furthermore, certain buffer systems, e.g. phosphates or acetic acid/sodium acetate 55 are ecologically undesirable.

It has now been found that with the present process, which permits of a controlled adjustment of the pH

value from a higher value to a stable lower final value, it is possible to achieve clearly better reliability in respect of surface levelness, reproducibility in shade of colour, depth of colour and degree of differentiation. This results in an appreciable reduction of the effective average dyeing time and in a simplification of the process. The final pH value can moreover be freely chosen and maintained constant, so that consequently there is much greater flexibility with respect to choice of dyes.

10 Besides the dyes, the dye bath may contain additives which influence the properties of the textile material, e.g. levelling agents, softening agents, antistatic agents, antioxidants, antimicrobial agents, additives producing a flameproof finish or improving the hydrophilic properties, and dirt-, water- and oil-repelling agents, additives for increasing fastness to wet-processing as well as antifoam agents.

The dyeing process according to the invention is performed preferably at elevated temperature, especially at 65° to 100° C. It is however also possible to dye in pressure-tight apparatus at a temperature up to 140° C., preferably at 100° to 120° C.

20 In general also circulation dyeing apparatus or circulation dyeing machines, such as jet dyeing machines, circulation apparatus for yarn or wound packages, beam dyeing machines, pack dyeing machines, winch vats or dyeing aggregates, onto which is constructed specifically for the said purpose an external circulation system, can be used for the process according to the invention.

25 The procedure is for example such that dyes and, optionally, an anionic auxiliary are added to the cold bath and, by means of the dosing device, alkali is allowed to flow into the bath until the desired initial pH value (6 to 12) is obtained; the textile material is then fed in and the bath is heated to the dyeing temperature, preferably 90° to 100° C. The procedure can however be reversed by firstly introducing into the dyeing apparatus the alkaline dye liquor together with the textile material to be dyed, and then adding the dyes and, 30 optionally, auxiliaries.

35 During the absorption period, the pH value can for example be maintained constant by means of the dosing device. After attainment of the dyeing temperature, dyeing is performed for 5 to 60 minutes, preferably for about 30 minutes. The pH value is then lowered by means of the dosing device to the final value (7 to 3.5) within 5-90 minutes. The acid preferably used is sulphuric acid. The dyes are practically completely absorbed, e.g. to the extent of over 99%, onto the textile material. This is removed, e.g. after cooling, preferably however at the dyeing temperature, from the dyeing apparatus and subsequently finished, e.g. without rinsing, by centrifuging, by subjecting it to suction or by 40 drying.

45 Into the used, preferably hot, dye liquor are now introduced dyes, optionally auxiliaries, and, by means of the dosing device, alkali. After attainment of the desired initial pH value, textile material is again fed into the dyeing apparatus and the dyeing process described above is repeated.

50 In principle the liquor can be used in this manner as often as desired. Preferably, however, it is discarded after 2 to 6 applications, since possibly difficulties can arise, e.g. due to the removal of dressing or brightening agents, marking inks or impurities from the textile material, or due to the accumulation of fluff.

As a result of the almost complete absorption of the dye, it is possible to use for the second application of the liquor dyes other than those used for the first dyeing. Preferably, however, the lightest dyeings in each case will be performed first.

The present invention concerns, apart from the dyeing process, also an apparatus for performing this process. This comprises a suitable dyeing aggregate, on which are provided arrangements which enable the pH value of the dye liquor to be measured, and also at least one dosing device by means of which additives can be introduced into the dye liquor, such as, in particular, the acid and alkali required for carrying out the process according to the invention. Preferably, both the pH-measuring points and the dosing devices are connected to an external liquor-circulation system, with the pH-measuring points being located in the direction of flow in front of and/or behind a dosing device.

In a preferred arrangement of the apparatus according to the invention, the external liquor-circulation system consists of several separate pipe lines which are joined in front of the point of discharge into the dyeing apparatus; and the inoculating point, at which the dosing device is connected to the liquor-circulation system, is located at the point at which the individual pipe lines join, with this dosing device being so designed that, by means of a controlled pump, an initial pH value can be obtained by the regulated addition of a strong alkaline solution and subsequently, by means of a controlled pump (closed loop control) giving a measured addition of a strong acid, the pH value can be lowered, after a predetermined function of time, to a final value.

The dosing device can however be connected at another point to the liquor-circulation system, and the dosing device and the pH-measuring point can be situated both on the same pipe line and on different pipe lines of the liquor-circulation system.

It is obvious that the described types of apparatus merely constitute exemplified embodiments, and that the dyeing process can be carried out also with other types of apparatus.

The following Examples serve to illustrate the invention without its scope being limited to them. The quantity values in the case of the dyes and auxiliaries relate to commercial material, and the temperatures are in degrees Centigrade.

#### EXAMPLE 1

A laboratory winch vat having a working width of 55 centimeters and a capacity of 500 liters is equipped with an external liquor-circulation system. The liquor is drawn up from the bottom of the vat and, by means of a pump, is fed through a pipe line, which is fitted with a flowmeter, back to the winch vat at its front end. Between the drawing-off outlet and the pump there are provided in the pipe line three drilled holes. Into the first hole in the flow direction is inserted a combined glass electrode. The second hole is connected via a tube direct to the dosing pump, and onto the third hole is mounted an additive container with tap, through which dye and solutions of chemicals can be introduced.

The winch vat is charged with a piece of polyamide-6 velvet pile carpet (Allyn 707), 50 cm in width, 23 m in length and 6.45 kg in weight, as well as with 240 liters of cold softened water. The turning rate of the carpet material is 12 meters per minute, and the delivery of the pump for the external liquor circulation is adjusted to 3600 liters/hour.

From the container there are added to the liquor, whilst this is heated with steam directly to 80° to 85°, 100 ml of 1 N sodium hydroxide solution and subsequently 96.75 g of the surface-active agent of the formula



dissolved in 1 liter of water, whereupon the pH value is 10.5.

There are then introduced from the additive container, within 10 minutes, 4.84 g of the yellow dye of the formula I



15 and 1.61 g of the blue dye of the formula II



25 both dissolved in 1.5 liters of water. The temperature of the liquor is simultaneously raised by means of direct and indirect steam to 93° to 96° and is subsequently maintained at this level.

30 Ten minutes after this temperature has been reached and the dyes have been added, a controlled addition is made by means of the dosing pump, at a rate of 50 ml per minute, of 1200 ml of 1 N sulphuric acid. The pH value of the liquor is afterwards 3.9. It increases during the next 10 minutes to 4.4. The liquor is practically exhausted, i.e. the dyes are absorbed to the extent of over 99%. The heating is shut off and the bath is cooled to 60° by opening of the winch vat and indirect cooling.

35 The carpet material is removed from the winch vat and, without rinsing, centrifuged and dried. It is evenly dyed light green.

40 Into this used liquor, which has a temperature of 58° and in which the loss of liquor has been approximately compensated for by the direct-steam condensate, is introduced, after the addition of 500 ml of 1 N sodium hydroxide solution and 98.25 g of an anionic levelling agent having affinity for the fibres, 6.55 kg (0.5×23 m) of the same carpet material. The pH value of the liquor is 11.2. The turning rate of the carpet material is again 12 meters per minute and the liquor-circulation rate is adjusted to 4800 liters per hour.

45 The bath is now heated within 10 minutes to 93° to 96°; and there is then introduced by means of the additive container, in the course of 6 minutes, a solution of 4.91 g of the dye of the formula I and 1.64 g of the dye

of the formula II in 1.5 liters of water. The temperature of the liquor is kept at 93° to 96°.

After a further 10 minutes is added by means of the dosing pump, at a rate of 20 ml per minute, 570 ml of 1 N sulphuric acid. The pH value of the liquor after the dosing pump has been turned off is 3.9, but increases to 4.25 in the course of the next 10 minutes. The dyes are absorbed onto the carpet material to the extent of over 99%. The liquor is cooled to 65°, the carpet material is removed from the winch vat and, without rinsing, centrifuged and dried. It is evenly dyed light green and cannot be distinguished in depth of colour and in shade from the material firstly dyed.

Into the liquor already used twice is introduced 5.94 kg (0.5 × 18 m) of an uncut pile carpet material, the loops of which are composed of a 50:50 mixture of basic dyeable polyamide (Antron 3 type 754) and deep-dyeing polyamide (Antron 3 type 757). There is then added at 60°, through the additive container within 5 minutes, 59.4 g of a nonionic levelling agent having affinity for the dyes (alkylamine polyglycol ether), dissolved in 1 liter of water, with the turning rate of the carpet being 12 m per minute and the circulation rate of the liquor 4800 liters per hour. The bath is heated within 15 minutes to 93° to 96° and kept at this temperature. During the heating up, 500 ml of 1 N sodium hydroxide solution is added; and on attainment of the final temperature are added in the course of 8 minutes, by way of the additive container, 20.79 g of the dye of the formula I, 8.91 g of the dye of the formula II and 3.56 g of the red dye of the formula III

(III)



dissolved in 1 liter of warm water. There are subsequently added in the form of their dispersions, diluted in 1 liter of water and fed in from the additive container, 65.34 g of the yellow dye of the formula IV

(IV)



0.71 g of the red dye of the formula V

(V)



and 2.67 g of the blue dye of the formula VI



(VI)

10 After 10 minutes is added by means of the dosing pump, at a rate of 20 ml per minute, 580 ml of 1 N sulphuric acid. The pH value of the liquor 10 minutes after completing the addition of the acid is 4.1. After cooling to 60° C., the liquor is drawn off and the carpet material is rinsed in the winch vat with 200 liters of water at 50° for 15 minutes. The carpet material is removed from the winch vat, centrifuged and dried. The result obtained is a level differential dyeing in an olive and golden-yellow shade.

#### EXAMPLE 2

A beam dyeing machine (laboratory piece-dyeing machine, Model 10, Rudolf Then) consists with regard to its main parts of the horizontal dyeing vat with cooling jacket, which vat is connected with the auxiliary vat by way of a special return pump to form a circulation system.

25 Into this dyeing machine is introduced a piece beam charged with a polyamide-6 uncut pile carpet material, 50 cm in width, 135 cm in length and 380 g in weight. Six liters of softened water and 60 ml of 2 N sodium hydroxide solution are fed into the auxiliary vat. By opening of the appropriate valves (auxiliary vat, or connecting pipe, pump/dyeing vat) the liquor flows by its own drop from the auxiliary vat into the dyeing vat, with the expelled air passing through the vent pipe to the auxiliary vat. After filling of the dyeing vat, there remains in the auxiliary vat a liquor residue to a depth of about 5 cm; the circulation pump is then switched on. For measurement of the pH value, a drilled hole had been provided in the piping between the dyeing vat and auxiliary vat (flow direction) and a combined glass electrode inserted. The dye liquor circulates during the entire dyeing process from the inside to the outside, during which process the pressure drop is 0.1–0.2 bar and the delivery of the pump is about 6 liters per minute. The liquor is heated to 98° and 7.6 g of an anionic levelling agent having affinity for the fibres, dissolved in 100 ml of water, is fed in the course of 5 minutes into the auxiliary vat.

30 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9



(VIII)

changed. Level dyeings are obtained which, in shade and depth of colour, do not differ from the first two dyeings.

## EXAMPLE 3

The piece beam of the beam dyeing machine (see Example 2) is wound with a polyamide-6.6 serge filament fabric, which is fixed and bleached,  $20 \times 0.5$  m in size and 670 g in weight. This piece beam is introduced into the dyeing vat. Six liters of cold softened water and 12 ml of 1 N sodium hydroxide solution are fed into the auxiliary vat. A combined glass electrode (see Example 2) enables the pH value to be measured. The liquor is subsequently transferred, as described in Example 2, to the dyeing vat, and 6.7 g of the same levelling agent is added. The dyeing temperature is adjusted to 97° to 98° and the pH value is 9.4.

5 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000

5.36 g of the dye of the formula I, 2.28 g of the dye of the formula II and 2.28 g of the dye of the formula III according to Example 1, together dissolved in 200 ml of hot water, are fed in the course of 10 minutes from a dropping funnel into the auxiliary vat. After 15 minutes, an addition is made by means of a flask burette, at a rate of 2.5 ml per minute for 20 minutes, of 50 ml of 1 N sulphuric acid.

The pH value after a further 10 minutes is 4.2. The dye bath is exhausted, i.e. the dyes have been absorbed to the extent of over 99% onto the material being dyed. The heating is switched off and, with the aid of indirect cooling, the dye liquor is cooled to 60°. The liquor, almost as clear as water, is pumped back into the auxiliary vat and the piece beam is taken out. The filament fabric is unwound, dewatered by squeezing and dried. The fabric is evenly dyed in a green shade.

The used liquor, which is at a temperature of 55°, is made up with 900 ml of softened water again to 6 liters, thus compensating for the loss of liquor. The piece beam is wound with 670 g ( $20 \times 0.5$  m) of the same polyamide-6.6 serge filament fabric and introduced into the dyeing machine. As in the case of the preceding dyeing of this Example, the liquor is subsequently transferred to the dyeing vat, and thereupon the same amount of levelling agent is added. The dyeing temperature is brought to 97° to 98°.

5 10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000

5.36 g of the dye of the formula I, 2.28 g of the dye of the formula II and 2.28 g of the dye of the formula III, together dissolved in 200 ml of hot water, are fed in the course of ten minutes from a dropping funnel into the auxiliary vat. After a further 15 minutes, an addition is made by means of a flask burette, for 25 minutes at a rate of 1.4 ml per minute, of a total weight of 35 ml of 1 N sulphuric acid. The pH value after a further 10 minutes is 4.1. The pH value is continuously checked by means of the combined glass electrode incorporated into the circulation system.

The dye bath is exhausted, i.e. the dyes have been absorbed to the extent of over 99% onto the material being dyed. The heating is switched off and, with the aid of indirect cooling, the dye liquor is cooled to 60°. The almost colourless liquor is pumped back into the auxiliary vat and the piece beam is taken out. The filament fabric is unwound, dewatered by squeezing and dried.

The polyamide fabric is evenly dyed and, with regard to depth of colour and shade, does not differ from the dyeing carried out initially.

both dissolved in 200 ml of hot water. After 30 minutes, an addition is made by means of a flask burette, for 10 minutes at the rate of 5.5 ml per minute and for a further 20 minutes at the rate of 2.25 ml per minute, of a total amount of 100 ml of 1 N sulphuric acid.

The pH value after a further 10 minutes is 3.8. The dye bath is exhausted, i.e. the dyes have been absorbed to the extent of over 99% onto the material being dyed. The heating is switched off and, with the aid of indirect cooling, the dye liquor is cooled to 60°. During this time the pH value increases to 3.9. The liquor, almost as clear as water, is pumped back into the auxiliary vat and the piece beam is taken out. The carpet material is unwound, centrifuged and dried. The polyamide-6 loop pile carpet material has been evenly dyed in a green shade.

The used liquor, which is at a temperature of 55°, is made up with 600 ml of softened water again to 6 liters, thus compensating for the loss of liquor. The piece beam is wound with 380 g ( $50 \times 135$  cm) of the same polyamide-6 loop pile carpet material and is introduced into the dyeing machine. After the addition of 63 ml of 1 N sodium hydroxide solution to the liquor, the pH value is 11.0. The liquor is subsequently transferred as in the case of the preceding dyeing to the dyeing vat and, in the same manner, the identical amount of levelling agent is added. The dyeing temperature is adjusted to 97° to 98° and the pH value is 10.2.

2.28 g of the dye of the formula VII and 1.52 g of the dye of the formula VIII, both dissolved in 200 ml of hot water, are now fed from a dropping funnel, within 10 minutes, into the auxiliary vat. After a further 30 minutes, an addition is made by means of a flask burette, for 10 minutes at a rate of 5.5 ml per minute and for a further 20 minutes at a rate of 1.4 ml per minute, of a total amount of 73 ml of 1 N sulphuric acid. The pH value after a further 10 minutes is 3.9. The pH value is continuously checked by means of the combined glass electrode mounted between the dyeing vat and auxiliary vat. The dye bath is exhausted, i.e. the dyes have been absorbed to the extent of over 99% onto the material being dyed. The heating is switched off and, with the aid of indirect cooling the dye liquor is cooled to 60°, during which time the pH value has risen to 4.0. The almost exhausted liquor is pumped back into the auxiliary vat and the piece beam is taken out. The carpet material is unwound and, without being rinsed, is centrifuged and dried. The polyamide-6 loop pile carpet material is evenly dyed in a green shade and, with regard to depth of colour and shade, does not differ from the initially dyed carpet material.

Corresponding to this second dyeing, two further dyeings are performed on the same polyamide-6 carpet material, with small differences in weight being taken into account in fixing the weighed amounts of dyes and auxiliaries. The applied amounts of 1 N sodium hydroxide solution and also the dosing rates for the flask burette, which again contains sulphuric acid, are un-

## EXAMPLE 4

The apparatus shown in drawing 1 comprises a carpet winch vat (make "Brückner" type HKP, capacity max. 25.4 m<sup>3</sup>, working width 5 m), which is provided with an external liquor circulation system. From the dyeing apparatus 1, the liquor is pumped through the suction piping 2 by means of the circulation pumps 3 and through the pipes 4 back to the dyeing apparatus, with a liquor-distributor with a spreading-trough 5 ensuring that the liquor on re-entering the dyeing apparatus is distributed as evenly as possible over the width of material. Into the pipes 4 are incorporated heat exchangers 6, a pH-measuring point 7—consisting of reference electrode type 8423 and glass electrode type 8403 (make "Polymetron"), previously calibrated at 20° by means of buffer solutions at the values of 4.00, 7.00 and 10.00—as well as a dosing device 8. This consists, as is shown by drawing 2, of a storage tank 9, which is connected, by way of a shut off valve 10, a pump 11 (make "Bran & Lübbe", type Normados NK 31), a nonreturn valve 12, a further shut off valve 13 and an inoculating point 14, to the pipe 4. In addition, the dosing device is fitted with a safety valve 15.

The winch vat is filled to the extent of 80% with 25 works water, and the water temperature in the vat is 18°. There are introduced into the vat 2 liters of anti-foam agent and then successively 4.4 liters of sodium hydroxide solution 38° Baumé and 7.1 kg of an anionic auxiliary, each diluted with about 100 liters of water. 64 30 g of the dye of the formula I, 32 g of the dye of the formula III and 48 g of the dye of the formula II according to Example 1 are thereupon dissolved, with stirring, in 300 liters of hot water containing 30 g of Calgon dissolved, and quantitatively fed into the winch vat. After dyes, auxiliaries and chemicals have become well dispersed in the course of 5 minutes, a 220 meter length of polyamide-6.6 velvet pile carpet material having a width of 5 meters (carrier material: polypropylene strips) and a total weight of 710 kg is introduced into the 40 winch vat. The winch speed is adjusted to 70–75 meters per minute, and the circulation rate of the liquor is between 6 and 7 cubic meters per minute.

The winch vat is allowed to run for 10 minutes without heating. It is then heated within 30 minutes to 90° 45 and dyeing is performed for a further 30 minutes at 90° in order to ensure a uniform distribution of the dyes. The pH value of the liquor is 9.0, and the degree of exhaustion of the dyes is about 70%. By means of the dosing pump, 1 M sulphuric acid is added at the rate of 1.9 liters per minute for 18 minutes, after which time the pH value is 6.7, rising however in the next ten minutes to about 7.5. Samples are taken after 10 minutes, by which is established that there is no trace of unevenness (difference right side-middle-left side). This test takes 9 55 minutes. There are thereupon added, for 10 minutes at a rate of 0.95 liter per minute, then for 5 minutes at a rate of 1.6 liters per minute, and finally for 5 minutes at a rate of 2.5 liters per minute, 1 M sulphuric acid up to a pH value of the liquor of 4.2. After a further 5 minutes, 60 there are again taken 3 samples which correspond, in shade and depth of colour to the production standard. The liquor is practically completely exhausted.

The liquor is now cooled by means of indirect cooling to 55° to 60°, and thereupon cooled to 43° by the 65 addition of 20% of fresh water. The carpet material is run out, taken off and passed direct to the dryer. The dried carpet material is shown to be dyed in a level

light-beige shade. As a result of the removal of the carpet material, about 1/5 of the amount of liquor is taken out with it. To the liquor at 43° are then added 2 liters of antifoam agent and 4.9 liters of sodium hydroxide solution of 38° Baumé, but the same amount of the anionic auxiliary and dyes. The measurements, type and weight of the carpet material are the same as those in the case of the first dyeing. The procedure carried out is essentially the same as that for the first dyeing, whereby the heating time and the dosing times were insignificantly shorter. The evenly dyed carpet material has a depth of colour and a shade which are identical to those of the first batch of material.

There are again introduced 2 liters of antifoam agent, 15 4.9 liters of sodium hydroxide solution 38° Baumé and this time 10.5 kg of the anionic auxiliary into the used liquor now at 44°. Into the winch vat are then fed 604 g of the dye of the formula I, 270 g of the dye of the formula III and 380 g of the dye of the formula II, dissolved in about 300 liters of hot water containing 30 g of Calgon. The identical carpet material which is then introduced weighs 712 kg. The procedure carried out is basically the same as that in the case of the beige batch first described. The dried carpet material is dyed evenly in a lighter-brown shade.

The amount of water consumed in the winch vat in performing these three dyeings (without reckoning the cooling water for the indirect cooling of the liquor) is less than half the amount required for the same carpet dyeings when dyeing is performed by conventional processes. Furthermore, the content of organic substances in the waste liquor is very low.

It goes without saying that this method of procedure is scarcely feasible for production practice without an 35 automatic system of control, since a continuous monitoring and adjusting of the pH value, of the dosing rate, etc., is necessary during the course of the process.

## EXAMPLE 5

The apparatus shown in drawing 1 comprises a carpet winch vat (make "Brückner" type HKP, capacity max. 21.4 m<sup>3</sup>, working width 4 m), which is provided with an external liquor-circulation system. From the dyeing apparatus 1, the liquor is pumped through the suction piping 2 by means of the circulation pumps 3 through the pipes 4 and back to the dyeing apparatus, with a liquor distributor fitted with a spreading-trough 5 ensuring that the liquor on re-entering the dyeing apparatus is distributed as evenly as possible over the width of material. Into the pipes 4 are incorporated heat exchangers 6, a pH-measuring point 7—consisting of reference electrode type 8423 and glass electrode type 8403 (made "Polymetron"), previously calibrated at 20° by means of buffer solutions at the values of 4.00, 7.00 and 10.00—as well as a dosing device 8. This consists, as is shown by drawing 3, of a storage tank for acid 9, which is connected, by way of a shut-off valve 10, a pump 11 (make "Bran & Lübbe", type Normados NP 41), a nonreturn valve 12, a further shut-off valve 13 and an inoculating point 14, to the pipe 4.

On the storage tank for sodium hydroxide 23 is mounted a circulation pipe system with shut-off valve 24, pump 25 and reducing valve 26. From the circulating flow of alkaline solution there is fed, by means of a magnetic valve 27 controlled by the alkaline-solution controller 28, into the liquor-circulation system in pipe 4 the amount of alkaline solution necessary for the attainment of the initial pH value. The alkaline-solution

controller receives the set point for the initial pH value from the set point programmer 22 and the actual level of the pH value from the electrodes 16, located in the pipe 4, via the measured-value transmitter 17. The actual value of the pH can be observed on the measuring instrument 18. The set point of the pH can be adjusted on the set point programmer 22 and also read off. The control of the acid pump 11 is effected by the controller 19 by means of a control motor 20, which, at constant stroke frequency, continuously adjusts the stroke between 0 to 100%. This controller receives the set point for the pH value, falling with increasing time, from the set point programmer 22, the actual value for the pH from the electrodes 16 via the measured-value transmitter 17, and the actual value of the pump-stroke setting 15 from the position-feed-back potentiometer 21. The actual value of the pH at any time can be observed on the measuring instrument 18. The set point of the pH at any time can be read off on the set point programmer 22.

The operating part of the desired-value controller 20 shown in drawing 4 consists of the following operating elements, which fulfill the following functions:

| Designation                            | Function                                                                       |
|----------------------------------------|--------------------------------------------------------------------------------|
| rotary knob with indication "pH-start" | 30 setting of the pH value at start of dyeing                                  |
| press button "start alkaline solution" | 31 starting of the alkaline-solution dosing device                             |
| press button "stop alkaline solution"  | 32 stopping of the alkaline-solution dosing device                             |
| indication "pH actual"                 | 33 indication of the instantaneous pH value in the dye liquor                  |
| indication "pH set point"              | 34 indication of the pH set point                                              |
| rotary knob with indication "G 1"      | 35 setting of the pH gradient 1 ( $\text{pH} \cdot 10^{-1} \text{ min}^{-1}$ ) |
| rotary knob with indication "pH-mean"  | 36 setting of the pH value at which switching to "G 2" occurs                  |
| rotary knob with indication "G 2"      | 37 setting of the pH gradient 2 ( $\text{pH} \cdot 10^{-1} \text{ min}^{-1}$ ) |
| rotary knob with indication "pH-final" | 38 setting of the pH value at end of dyeing                                    |
| press button "start acid"              | 39 starting of the acid-dosing device                                          |
| press button "stop acid"               | 40 stopping of the acid-dosing device                                          |

Pilot lamps incorporated into the press buttons and mounted adjacent to the rotary knobs indicate the current status of the functions of the set point programmer. 40

Dyeings are performed analogously to Example 4 using this control and regulating apparatus. In the following are merely described details which relate to the control and regulating apparatus. The type and amounts 45 of the dyes, auxiliaries and carpet material are analogous to those in Example 4.

The vat is charged with cold water, auxiliaries and dyes; the circulation pumps are allowed to run for 5 minutes; the alkaline-solution dosing device is then 50 switched on, the apparatus is allowed to run for 10 minutes without heating, and subsequently the carpet material is introduced and the heating is switched on.

The initial pH value of 8.5 previously set on rotary knob 30 is reached after 15 minutes. The dyeing temperature of 95° is attained after a further 25 minutes, and the alkaline-solution dosing device is shut off. After a subsequent migration phase of 20 minutes, samples are taken and then the acid dosing device, with a value of 0.075  $\text{pH min}^{-1}$  adjusted on press button 35, is started. 60 After a further 40 minutes, the "pH average" of 5.5 is attained, and the set point programmer switches over to the more rapid dosing rate G2 (button 37) of 0.1- $\text{pH min}^{-1}$ . The final pH value of 3.5, set on press button 38, is reached after 20 minutes and is maintained until after 65 sampling. After switching off the dosing device, the carpet is removed from the hot liquor and finished in the usual manner. The result is a level dyeing. The

liquor is practically completely exhausted. As in Example 4, the dye liquor can be re-utilised. In further dyeings using this procedure, the gradients G1 and G2 are varied from 0.05 to 0.2  $\text{pH min}^{-1}$ , and hence the effective dyeing times are varied between 1.5 hours and 3.5 hours.

Compared with the dosing device used in Example 4, the embodiment described above has the advantages that operating the apparatus is considerably simplified, and that the closed-loop control with programmed set point of the pH value is clearly less influenced by interference effects such as varying quality of water, concentration of acid and alkaline solution, and other similar factors.

#### EXAMPLE 6

A winch vat (make "Brückner" type H.K.P., capacity max. 21.4  $\text{m}^3$ ) is filled to the extent of 80% with works water. The water temperature is 18°. Into the vat are fed 2 liters of antifoam agent and subsequently 5.75 kg of a nonionic auxiliary (alkylaminopolyyglycol ether), diluted with 100 liters of water.

The following are then dissolved with stirring in 300 liters of hot water:

1344 g of the dye of the formula I,  
422 g of the dye of the formula II,  
721 g of the dye of the formula III,  
46.1 g of the dye of the formula IX



12.7 g of the dye of the formula X



and 12.7 g of the dye of the formula XI



and the solution is quantitatively introduced into the winch vat. The pH value is simultaneously adjusted to 8 by the controlled addition (for dosing device see Example 5) of 2 N sodium hydroxide solution. After dyes, auxiliaries and chemicals have become well dispersed within 5 minutes, a 260 meter length of polyamide-6.6 loop pile carpet material having a width of 4 meters and a total weight of 575 kg (carrier material: polypropylene strips), the loop pile of which is a 50:50 mixture of basically dyeable polyamide (Antron III, type 754) and deep-dyeing polyamide (Antron III, type 757), is fed into the winch vat. The rotational speed is adjusted to 70-75 meters per minute. The liquor circulation is 6 to 7 cubic meters per minute. The winch vat is allowed to run during 5 minutes without heating. The temperature is then raised within 35 minutes to 94° C., and during this time the pH value of 8 is kept constant (measured at the respective temperature) by the controlled addition (dosing) of 2 N sodium hydroxide solution. After attainment of the final temperature, the dosing device is switched off and dyeing is subsequently performed at this temperature (94° C.) for 30 minutes in order to ensure a good surface levelness. Three samples are taken at the end of this phase to check the evenness of the dyeing (difference: right side—middle—left side). No differences of shade are found. By means of the dosing device (see Example 5), the pH value is lowered with 1 N sulphuric acid linearly from 8 to 6 within 40 minutes and from 6 to 3.5 within 15 minutes. Samples are taken after 10 minutes of pH stabilisation. The shade of colour (red-brown/beige), the depth of colour and the differentiation effect correspond exactly to the production sample. The dyebath is practically completely exhausted. The carpet material is now run out hot, taken off and passed directly to the dryer. The carpet material has a perfectly satisfactory surface levelness.

#### Re-utilisation

About 15 to 20% of the amount of liquor is lost with the carpet material on removal of this from the dyeing apparatus. This loss is made up by the addition of fresh water. There are again added to the liquor at 75° C., 2 liters of antifoam agent and subsequently 6.2 kg of the nonionic auxiliary (alkylaminopolylglycol ether), diluted with about 100 liters of water. The following are then dissolved or dispersed in 300 liters of hot water with stirring:

2439 g of the dye of the formula I,  
1045 g of the dye of the formula II,  
418 g of the dye of the formula III,  
7667 g of the dye of the formula IV,

83 g of the dye of the formula V and  
313 g of the dye of the formula VI,  
the resulting solution is quantitatively fed into the winch vat and the pH value is simultaneously adjusted to 8 by means of the controlled addition (dosing) of 2 N sodium hydroxide solution. After dyes, auxiliaries and chemicals have become well dispersed in the course of 5 minutes, a 285 meter length of polyamide-6.6 loop pile carpet material having a width of 4 meters and a total weight of 620 kg (same quality as in the case of dyeing 1) is introduced into the winch vat. The procedure carried out is essentially the same as that for the first dyeing, with it being possible however to reduce the heating-up time to about 10 minutes. The final pH value of the dyeing is adjusted to 4.1 and, after 10 minutes' pH stabilisation, samples are taken. The samples correspond in shade of colour—olive/golden-yellow—in the depth of colour and in the differentiation effect exactly to the production sample.

In consequence of the relatively high amounts of disperse dyes used, a complete exhaustion of the dyes is not possible in this case; no further re-utilisation of the liquor is therefore undertaken. The carpet material displays a fully satisfactory surface levelness.

We claim:

1. In a process for the level dyeing of synthetic polyamide textile material by exhaustion in an aqueous dyebath using an anionic, metal-free, non-fiber-reactive dyestuff, the improvement which comprises (1) contacting the textile material with the dyebath at a pH value in the range of 6 to 12, (2) during the dyeing, exhausting the dyestuff onto the textile material by lowering the pH by at least one pH unit by the addition of an inorganic acid having a  $pK_a$  value of less than 3.8 at 20° C., (3) separating the dyed textile material from the exhausted dyebath (4) adding to the exhausted dyebath additional dyestuff and sufficient alkali to adjust the dyebath pH value to the range of 6 to 12, and (5) repeating steps (1) and (2).
2. The process of claim 1, wherein the synthetic polyamide textile material is carpeting.
3. Process according to claim 1, wherein the acid is added continuously at a constant rate.
4. Process according to claim 1, wherein the acid is added continuously at different rates.
5. Process according to claim 1, wherein the addition of acid is periodically discontinued.
6. Process according to claim 1, wherein the acid is so added that a constant change of the pH value relative to time or temperature occurs in such a manner that one or more linear or nonlinear gradients result.
7. Process according to claim 1, wherein sulphuric acid is used.
8. Process according to claim 1, wherein at the commencement of dyeing the pH value is brought to the initial value by the controlled addition of a strong alkaline solution.
9. Process according to claim 8, wherein there is used an alkaline solution of which the  $pK_a$  value at 20° C. is above 9.2.
10. Process according to claim 1, wherein the bath is used two to six times.

\* \* \* \* \*